

Aug. 23, 1960

J. W. SMITH

2,950,214

CAST COATED PAPER AND METHOD OF MAKING THE SAME

Filed March 25, 1957



INVENTOR.  
JOHN W. SMITH

BY

*John V. Stein*

ATTORNEY.

2,950,214

CAST COATED PAPER AND METHOD OF  
MAKING THE SAMEJohn W. Smith, Chillicothe, Ohio, assignor to The Mead  
Corporation, Dayton, Ohio, a corporation of Ohio

Filed Mar. 25, 1957, Ser. No. 648,227

15 Claims. (Cl. 117—64)

This invention relates to the production of high gloss coated papers. More particularly, it relates to a continuous method of providing an improved mineral or pigmented cast-coated paper having unusually high brightness and high gloss, a high degree of opacity and good affinity for printing inks. And it incorporates the principle of coagulating certain coating adhesives to obtain a coated paper having improved optical properties not hitherto associated with cast-coated paper.

An early proposal for producing a glossy mineral-coated paper embodied the application of an aqueous mineral coating composition to a paper web, immediately pressing the wet coated surface into contact with a polished chromium drum surface, drying the coating while it remained in such contact and then stripping the coated paper from the drum surface. This proposal was first referred to as a calendering rather than a coating operation and the mineral coated paper allegedly produced thereby was characterized as "cast surface" paper. The term "mineral-coated paper" related to a paper comprising a fibrous base having on one or both surfaces a continuous layer of mineral or pigment composition which covers the fibers of the base and fills the hollows between the fibers on the surface of the base, so that when the coated paper is pressed against a heated chromium drum surface while the coating is in a highly plastic condition, the coating is rendered comparatively non-plastic before it is removed from this surface. The mineral coating composition was applied to the paper in the form of an aqueous suspension of pigment (usually clay, satin white, etc.) and an adhesive or binding agent (usually casein or starch).

The use of starch or casein per se as pigment binders for cast-coated paper leaves much to be desired. For example, casein which is preferred to starch in preparing cast-coated paper, has the characteristics of slow water release and low drying rates, resistance to ink penetration, deleterious effects on brightness and opacity of the finished paper when present in the required quantities, and if heated too greatly during drying may show a loss of binding ability before or during drum finishing operations. Moreover, there are other disadvantages and glaring defects, such as having the coating surface stick to the drum finishing surface after drying thereon, having air bubbles and occasional particles of foreign matter in the coating to form dull spots, the formation of holes, cracks, and other defects in the cast surface of the paper, and the formation of edge beads of coating on portions of the drying drum which extend beyond the edges of the paper web, all of which result from attempts to carry out the aforementioned proposal for producing a glossy mineral-coated paper.

Subsequent proposals have been directed to methods for partially overcoming certain of these disadvantages and defects. For example, one patentee has suggested pooling surplus liquid "coating material" at the nip where the paper web is pressed into contact with a cast-

ing surface. Desirably, this surplus liquid coating washes backwardly against an incoming paper web and allegedly performs the functions of flooding depressions in the surface of the paper web which otherwise would become air pockets during the casting operation, rejecting foam and air bubbles in the coating, preventing foreign material from marring the coated paper surface, improving the distribution of coating on the paper web, reducing difficulties with beads of coating forming on the casting surface beyond the edges of the paper web, and additionally serves, together with the press roll pressure, to govern the final coat weight on the paper. However, a following patent, assigned to the assignee of the aforementioned surplus liquid-coating-material method, and relating to a method for continuously cleaning the edges of a casting drum face, indicates that cast-coating operation problems are still existent.

Instead of the proposed pool of surplus fluid coating material at the nip when the paper web is pressed into contact with a casting surface, still another process was advanced which allegedly eliminated the liability of trapping air between a drum and a coated paper surface applied thereto. This process involves applying a fluid coating to a moving paper web, pressing the freshly coated surface into contact with a chrome casting surface, and maintaining a circulating pool of water in the casting nip thereby formed. The water pool rewets the still wet coated surface, displaces air in shallow pockets which might become non-glossy areas on the finished sheet, and by continuously washing the edges of the casting drum, partly overcomes the problem of edge beads. However, if this process is operated with a sufficiently low pressure in the casting nip so that there is no redistribution of the coating itself, independently of the water pool, the required intimacy of contact between the surface of the coating and the chromium casting surface cannot be obtained. Operation pressures high enough to give this redistributing action, disperse a portion of the coating in the water pool, and certain of the suspended solids present in the coating composition are inherently transferred to the water pool which thereby becomes milky in appearance. Some edge bead problem therefore persists and an appreciable quantity of the coating initially applied to the paper is lost to the sewer drain, and such loss is an obvious economic liability.

As previously pointed out, pigment binders for cast-coated paper cause the coating surface to stick and not completely release from the finishing surface, thereby effecting surface defects in the ultimate cast-coated paper product or preventing operations entirely. As a proposed remedy, it has been suggested that release agents, such as a film of oleaginous material be applied to a chromium casting drum before and/or during the time that the coated sheet contacts the casting drum. The function of oleaginous material on a chromium casting drum, however, is necessarily dependent on continuously maintaining a required quantity on the drum and this is determined by a skilled operator who must carefully watch the finished paper as it leaves the chromium drum, and increase or decrease the amount of liquid oleaginous material on the chromium drum and/or in the coating color in order to obtain adequate release of the coated paper from the chromium casting surface.

None of these attempts to produce the desired cast-coated paper has proven entirely satisfactory. Now in accordance with the present invention there has been discovered a method for continuously producing mineral cast-coated paper having outstanding characteristics, which method is not subject to the disadvantages of the prior art processes.

Generally, the present invention comprises applying

an aqueous, pigmented coating composition containing a pigment binder to a paper web and thereafter passing the web carrying the coating through a coagulant bath. As a result, the binding or adhesive component of the freshly applied coating without substantial drying, is converted by the coagulant into a gel, but in accordance with the invention, the coagulant is applied in such a way as to prevent distortion of the coating film. After substantially complete gelation of the pigment binder, the coating is then passed over a press roll and transferred to a casting surface, as for example, a methyl silicone resin casting surface chemically bonded to a metal substrate. While a small amount of the coagulant solution may accumulate as a pool in the nip between the press roll and the casting surface, such a pool does not contain suspended solids and because of the gelled condition of the coating, none of the solids in the coating pass into the pool of coagulant solution.

It is accordingly an object of the invention to provide a cast-surfaced coated paper having improved optical properties.

Another object is to provide a cast-surfaced coated paper having unusually high brightness and opacity and high gloss.

Another object is to provide a cast-surfaced coated paper having an enhanced affinity for printing inks.

Still another object is to provide an improved method for continuously producing such a paper having said characteristics, which method facilitates ready release of the coating from the casting surface and decreases normal surface defects on the paper.

Another object is to provide a method of the foregoing type adapted to relatively high speed production.

Another object is to avoid operating defects, such as the occurrence of edge beads, associated with prior processes referred to hereinbefore.

Another object is to provide a method which is adapted to wide commercial utilization and which produces a cast-surfaced paper product that can be used widely.

Numerous other objects of this invention will more fully hereinafter appear.

The accompanying drawing portrays diagrammatically one arrangement of equipment which has been satisfactorily employed for practicing the present invention.

Referring to the drawing, the paper web to be coated is drawn from a roll 10 of suitable paper base stock, and the web 11, is led over guide rolls 12 and 13 to pass through the apparatus in the coating color applying zone. In this modification, the web passes through the nip of the coating application rolls 14, 15 where a predetermined amount of coating suspension is applied thereto and distributed with sufficient uniformity over the web surface to give the desired weight of coating material per unit area on the web.

The present invention permits the use of commonly used aqueous, pigmented coatings, containing only such pigments, adhesives and additives as are normally used in preparing pigmented coatings for printing. In other words, a normally adhesive coating material such as a suspension or colloidal solution of pigment and adhesive material in a suspending or solvent fluid is applied by such apparatus to the paper web but application thereof is desirably made in such a manner as to provide the coated side of the web with a smoothness that is substantially free of surface irregularities. And the present invention permits use of simple and effective coagulants whereby the adhesive component of freshly applied mineral coating without substantial drying, is converted into a gel in a manner so as to prevent undesirable distortion of the coating film. Moreover, while the cohesion properties of the adhesive coating material appear to remain undisturbed after the coagulant reaction, the coating nevertheless has its characteristics temporarily modified so that the adhesive tendency which would normally be effective between the coating material and a casting surface is so

greatly reduced, that the surface coating material does not adhere to the casting surface after drying, but nevertheless acquires the smoothed surface characteristics of the casting surface. In addition, there is no substantial or practically appreciable disturbance of the smoothed surface coating as it separates completely from the casting surface as a high gloss coated paper.

In practical operations, utilizing the invention and the apparatus illustrated, under commercial operating conditions, this modification of the coating prior to a finishing operation on a casting surface, is effected by coagulating the mineral surface coating, after the coating has been applied evenly to the paper web, but before the coating is brought into contact with the casting surface. In actual practice, satisfactory results have been obtained by the modifying and/or stabilizing action of this invention by wrapping the freshly coated paper, without substantial drying, coated side out, tightly around roll 16 which dips into the coagulant solution or bath contained in a tub 17. As illustrated, the coated paper is rolled into and out of the coagulating bath in such a way that the coagulant only contacts the coated surface of the paper web and is reactive with the coating from the time the coating material is first brought into contact with the coagulant, until substantially complete gelation of the coating adhesive has been effected. In this manner, distortion of the coating film is prevented and following gelation, the coated paper 11 is transferred by press roll 18, through nip 19 to a finishing roll 20 having a smoothly buffed methyl silicone casting surface, such as disclosed in co-pending application, Serial No. 635,974, filed January 24, 1957. Roll 20, which is heated, has its smooth silicone surface in contact with the stabilized but moldable coating until the coating spontaneously releases from the silicone surface after it is substantially completely dried and is thereafter removed by tension roll 21. The dried coated paper is thereafter rolled up on winder roll 22.

The accompanying drawing illustrates one form of apparatus for applying the desired quantity of coating smoothly to the web. To accomplish this result, the color solids should preferably be adjusted so that the coating is not too viscous for easy application, nor so dilute as to be incapable of forming a tough gel. Relatively high solids content coating suspensions, e.g. of the order of 45%-65% solids or more, have been used successfully and, as a general rule, the preferred percentage of solids in the coating is governed by the type and quantity of adhesive selected for the color. For example, higher adhesive contents require lower solids, and latex may be used at higher solids than protein adhesives. In the apparatus shown, the coating color is fed through a suitable supply line and by suitable means to one or more discharge pipes or nozzles, indicated diagrammatically at 23, and into the nip between rolls 15 and 24 which have the direction of rotation as indicated, the color forming a pool 25. Doctor 26, as shown, functions to maintain the pool in the aforesaid nip between rolls 15 and 24 and any suitable well known doctoring means may be employed. Color from pool 25 preferably is allowed to overflow at both ends of the nip, and is recirculated. Such overflow of the pool provides a means for removal of grit which otherwise would accumulate in the pool.

Roll 24 runs in contact with the application roll 15 and provides for metering thereon a regulated quantity of uniformly distributed coating material which in turn is transferred from roll 15 to the traveling web of paper as it passes through the nip of the application rolls 14, 15.

The coating apparatus shown is a reverse roll system and has been found to be very satisfactory and effective for transferring from the trough of coating material or so-called coating color, between rolls 15 and 24, accurately controlled amounts of the coating material. With high solids content coating colors of the order of as high

as 65% solids, which in their normal condition are substantially non-flowable, this apparatus, with the rolls under considerable pressures of the order of 10 to 100 pounds per lineal inch, and with roll 24 being operated at 0.1-0.5 times the speed of application roll 15 which was turned at from 1.38-3.00 times the speed of the paper web 11, effects a large temporary change from its normal condition of non-flowability, causing it to become readily

plastometer reading of the order of 80 to 140 P. & J. when measured with a  $\frac{1}{8}$  inch ball. And if one or more of these three rolls is hard surfaced, i.e., of metal, Stonite, or the like, then its adjacent roll is preferably resilient surfaced. For example, the following combinations of these coating mechanism rolls have been found commercially suitable and are presented in illustration but not in limitation of the invention.

| Roll No. | Type of Roll By Combination |                |                |                |                |
|----------|-----------------------------|----------------|----------------|----------------|----------------|
|          | (1)                         | (2)            | (3)            | (4)            | (5)            |
| 14-----  | Metal.....                  | 140 P & J..... | 136 P & J..... | 80 P & J.....  | 140 P & J..... |
| 15-----  | 112 P & J.....              | Metal.....     | 112 P & J..... | 130 P & J..... | Stonite.....   |
| 24-----  | Metal.....                  | 112 P & J..... | Metal.....     | 112 P & J..... | 112 P & J..... |

fluent and flowable so that it may be thus accurately controlled as to quantity and general distribution. The coating material passing in controlled amount through the nip of the rolls 15, 24 is carried on the surface of roll 15 as it travels up toward the paper web, to transfer the desired quantity of coating material for the predetermined coat weight desired, and in such condition of flowability that the color will be generally distributed across the surface of the roll 15 as it moves toward the paper and application nip of rolls 14, 15. In such condition of flowability and such distribution when brought in contact with the paper web by roll 15 turning in a direction opposite to the direction of travel of the paper web, there will be transferred to the web a substantially uniformly distributed layer or film of coating material which is of considerable and unexpected smoothness. The coating materials commonly used, contain a substantial amount of adhesive material such as casein. However, by the disclosed reverse roll system, there is sufficient working of the coating color both before it passes into the application nip of the rolls 14, 15, and also within the nip by reason of the reverse turning of roll 50, so that even high solids content coating colors will be made sufficiently fluid, for securing the desired accurate coat weight, and the uniform distribution of the film upon the surface of the paper web. Moreover, the apparatus referred to, when using somewhat lower solids content colors with greatly reduced viscosity and corresponding increased flowability, has been very satisfactory in applying the desired quantity and uniform distribution of coating material to the paper web, and of leaving a surface which is sufficiently smooth so that it may be subsequently coagulated and dried on a finishing surface to give the desired high gloss coated paper. In the latter case, rolls 15, 24 are preferably operated at a low pressure of the order of 10 pounds per lineal inch, or lower and may even be operated at a gap amounting to as much as .005 inch.

Again, referring to the coating apparatus illustrated, very satisfactory results have been attained when rolls 14 and 15 were rubber covered rolls; roll 14 having a plastometer reading of about 136 P. & J. and roll 15 having a plastometer reading of about 112 P. & J. Rolls 14 and 15 may be operated with a pressure therebetween varying during operation, for example from about 1 to 25 pounds per lineal inch, with satisfactory results having been obtained at a pressure of preferably about 10 pounds per lineal inch. Roll 24 in this connection was a hard surfaced Stonite roll. Rolls 18 and 21 had plastometer readings of 65 and 32 P. & J. respectively, while roll 20 was a metal roll, having a smoothly buffed methyl silicone casting surface, such as disclosed in copending application, supra. Roll 16 was a corrosion resistant roll such as stainless steel. More generally, however, it has been found that rolls 14, 15 and 24 may all be resilient surface type rolls, such as rubber covered rolls having a

20 All plastometer values were measured with a  $\frac{1}{8}$  inch P. & J. ball.

The pressure in operation between rolls 18 and 20 may be varied over a substantial range; for example, from about 50 to 150 pounds per lineal inch, with satisfactory results having been obtained at a pressure of about 75 pounds per lineal inch. In this connection, it has been found that the upper pressure limit is determined by the strength or toughness of the gelled coating. And the pressure between rolls 18 and 20 may be varied over wide limits so long as sufficient pressure is used to insure intimate contact between the coating surface and the casting surface.

Various coating materials may be employed in practicing the present invention and as indicated by the formulations hereinafter set forth, the coating material generally comprises a mineral and an adhesive in aqueous medium. Both the adhesive content and the total solids content of the coating materials to be used are predicated on the ultimate high gloss coated paper desired and for 35 highly satisfactory operations, such adhesive and total solids contents may be somewhat critical. For example, it has been found that the preferred range of adhesive contents is of the order of 12%-20%, although more or less adhesive can be used if special end-use requirements 40 of the ultimate high gloss paper product so dictate. Moreover, if starch is used in admixture in the adhesive, more total adhesive is required than if it is not so used. Generally, the higher region of the adhesive content range is useful in preparing papers for offset printing, 45 while the lower range has been found useful for letter-press printing.

A color formula which has been found to function satisfactorily in the practicing of the invention is of the following composition, wherein the parts by weight are 50 taken on a dry basis:

#### Example I

|                                                                                                                | Parts by weight |
|----------------------------------------------------------------------------------------------------------------|-----------------|
| Clay (English coating clay) -----                                                                              | 42.0            |
| 60 Calcium carbonate -----                                                                                     | 42.0            |
| Casein (Argentina) -----                                                                                       | 12.0            |
| Caustic soda (parts per 100 parts of casein) --                                                                | 6.0             |
| Sodium pyrophosphate -----                                                                                     | 0.75            |
| Calcium stearate -----                                                                                         | 0.5             |
| 65 Dow 512-R latex (butadiene-styrene copolymer 30:70) -----                                                   | 6.0             |
| Di-isobutylphenoxyethoxyethyldimethylbenzylammoniumchloride, monohydrate (Hyamine 1622, Rohm & Haas Co.) ----- | 0.05            |

70 Such color gives satisfactory results in the practicing of this invention when admixed with water to have a solids content of approximately 50.5%.

75 The following examples of color formulations which have likewise been used satisfactorily are set forth for

purposes of illustration, but not of limitation. The parts by weight of these compositions are taken on a dry basis:

## Example II

|                                                   | Parts by weight |
|---------------------------------------------------|-----------------|
| Clay (English coating clay)                       | 42.0            |
| Calcium carbonate                                 | 42.0            |
| Soya protein (refined)                            | 12.0            |
| Ammonia, 26° Bé. (parts per 100 parts of protein) | 12.0            |
| Dow 512-R latex                                   | 4.0             |
| Sodium pyrophosphate                              | 0.75            |
| Calcium stearate                                  | 0.5             |
| Hyamine 1622                                      | 0.05            |

## Example III

|                                                   | Parts by weight | 15 |
|---------------------------------------------------|-----------------|----|
| Clay (English coating clay)                       | 38.0            |    |
| Calcium carbonate                                 | 41.0            |    |
| Satin white                                       | 5.0             |    |
| Alpha protein                                     | 12.0            |    |
| Ammonia, 26° Bé. (parts per 100 parts of protein) | 12.0            |    |
| Dow 512-R latex                                   | 4.0             |    |
| Sodium pyrophosphate                              | 0.75            |    |
| Calcium stearate                                  | 0.5             |    |
| Lignasan                                          | 0.05            |    |

## Example IV

|                                                        | Parts by weight | 30 |
|--------------------------------------------------------|-----------------|----|
| Clay (English coating clay)                            | 51.0            |    |
| Clacium carbonate                                      | 30.0            |    |
| Alpha protein                                          | 18.0            |    |
| Azite (dicyandiamide) (parts per 100 parts of protein) | 25.0            |    |
| Ammonia, 26° Bé. (parts per 100 parts of protein)      | 12.0            |    |
| Sodium pyrophosphate                                   | 0.75            |    |
| Calcium stearate                                       | 0.5             |    |
| Lignasan                                               | 0.05            |    |

## Example V

|                                                   | Parts by weight | 35 |
|---------------------------------------------------|-----------------|----|
| Calcium carbonate                                 | 84.0            |    |
| Alpha protein                                     | 12.0            |    |
| Ammonia, 26° Bé. (parts per 100 parts of protein) | 18.0            |    |
| Dow 512-R latex                                   | 4.0             |    |
| Sodium pyrophosphate                              | 0.75            |    |
| Calcium stearate                                  | 0.5             |    |
| Hyamine 1622                                      | 0.05            |    |

## Example VI

|                                                        | Parts by weight | 45 |
|--------------------------------------------------------|-----------------|----|
| Clay (domestic coating clay)                           | 81.0            |    |
| Soya protein (refined)                                 | 12.0            |    |
| Azite (dicyandiamide) (parts per 100 parts of protein) | 25.0            |    |
| Ammonia, 26° Bé. (parts per 100 parts of protein)      | 15.0            |    |
| Sodium pyrophosphate                                   | 0.75            |    |
| Sulphonated tallow (Vegetol)                           | 1.0             |    |
| Calcium stearate                                       | 0.5             |    |
| Dow 512-R latex                                        | 7.0             |    |
| Hyamine 1622                                           | 0.1             |    |

Particularly satisfactory high gloss coated papers of the invention were produced by applying the coating of Example I, supra, to the web 11 as shown in the drawing. While the layer of coating was still sufficiently mobile or deformable, the web, coated side out, was tightly wrapped around roll 16, as shown, thereby rolling the coated paper into and out of the coagulating bath and concomitantly initiating gelling of the adhesive component of the coating. Roll 16 is so spaced from nip 19 as to permit substantially complete gelation during the time the coating on the web is treated with coagulant until the web is transferred by press roll 18 to the heated silicone resin finishing roll 20. In this instance, the coating, after coagulating but prior to casting, was in the form of a non-tacky, tough but deformable gel. And the resulting cast-coated paper had a Bausch & Lomb gloss of 86.0 and was without megoscopic surface defects, such as are frequently found in cast-surfaced coated papers. This paper also had enhanced affinity for print-

ing inks as compared to cast-surfaced coated paper not produced in accordance with this invention.

Even when using less expensive pigments such as domestic coating clay in color formulae when practicing this invention, it has been found that cast-surfaced coated papers have unexpectedly high brightness and opacity. In this connection, reference is made to the following chart which depicts typical brightness and opacity improvement of cast surface coated papers as attained by this invention, using the coagulating agents designated and the coating formula of Example VI, supra:

| Coagulating Agent<br>Used—all solutions<br>10% by weight solid<br>material | G.E. Brightness |                   | Bausch & Lomb TAPPI<br>Opacity |                   |
|----------------------------------------------------------------------------|-----------------|-------------------|--------------------------------|-------------------|
|                                                                            | Coagulated      | Not<br>Coagulated | Coagulated                     | Not<br>Coagulated |
| Aluminum Sulfate                                                           | 80.0            | 78.0              | 97.0                           | 96.0              |
| Zinc Sulfate                                                               | 89.2            | 78.3              | 97.5                           | 96.2              |
| Magnesium Chloride                                                         | 79.7            | 78.8              | 97.0                           | 96.3              |
| Calcium Chloride                                                           | 79.7            | 78.8              | 97.7                           | 96.3              |
| Zinc Chloride                                                              | 80.0            | 79.0              | 97.3                           | 96.1              |
| Barium Chloride                                                            | 80.5            | 77.7              | 97.0                           | 96.8              |
| Lead Acetate                                                               | 80.1            | 77.6              | 97.0                           | 96.2              |
| Zinc Acetate                                                               | 81.8            | 78.2              | 97.3                           | 96.2              |

G.E. brightness referred to herein is a measurement of the degree of reflectance of light from the paper surface as measured with a General Electric reflection meter.

Similarly, the table following shows that this unexpected improvement in both brightness and opacity is relatively insensitive to concentration of the coagulant solution in the practice of this invention to produce cast surface coated papers, using the coating formula of Example VI, and when treated with various concentrations of zinc acetate:

| Weight Percent<br>Zinc Acetate | G.E. Brightness |                   | Bausch & Lomb TAPPI<br>Opacity |                   |
|--------------------------------|-----------------|-------------------|--------------------------------|-------------------|
|                                | Coagulated      | Not<br>Coagulated | Coagulated                     | Not<br>Coagulated |
| 10.0                           | 79.3            | 75.0              | 96.9                           | 95.5              |
| 7.5                            | 80.1            | 75.9              | 97.3                           | 96.0              |
| 5.0                            | 80.0            | 75.4              | 97.0                           | 95.6              |
| 4.0                            | 79.7            | 75.6              | 97.1                           | 96.1              |
| 2.5                            | 79.8            | 75.7              | 96.9                           | 96.0              |

The toughness of the gel preferably is adjusted so that the coating is plastic enough to deform under the pressure applied at casting nip 19 yet tough enough so that absolutely none of the coating is removed in this nip. It has been found that proper gel toughness may be obtained by proper selection of an electrolyte within the group of preferred coagulants, by varying the coagulating bath temperature and concentration, and by altering the time of exposure of the coating to the reaction of the coagulant prior to casting. Selection of the coagulant depends upon the particular adhesive employed in the coating, but it should be a colorless, water-soluble electrolyte, which is neither a strong acid nor a strong alkali. As noted hereinbefore, these factors can be varied over wide limits without critically affecting the operation of the process. When starch is used alone, it is difficult to obtain a sufficiently tough gel to withstand the casting operation. When casein, soya protein, synthetic rubber latex and similar materials or their mixtures are used as the adhesive, or when mixed with less than an equal amount of starch, the soluble salts of polyvalent metals and weak organic acids perform best. The acetates, or formates of calcium, zinc, barium, lead and aluminum are preferred coagulants, because they function adequately to give the desired effects, yet do not reduce the pH of the finished paper too greatly. Sulfates, chlorides, and other strong acid salts of these metals may be used where an acid pH is not objectionable in the paper or when a highly alkaline mineral such as satin white is used in the coating color

in an amount sufficient to neutralize the residual acidity of the coagulant.

In general, it has been found that water soluble compounds within the group of calcium, zinc, barium, lead, magnesium, cadmium or aluminum salts of formic, acetic, citric, tartaric, lactic, hydrochloric and sulfuric acids provide suitable coagulants for this invention. Moreover, under certain conditions free organic acids such as lactic acid may be effective coagulants. And the concentration of the coagulant may, of course, be varied to compensate for its specific activity, the temperature of the coagulant bath and the speed of operation.

Generally, the more active coagulants produce the greatest optical improvement in the finished paper. Coagulant concentrations of from 1 to 20 percent by weight in water are useful, the preferred range being from 3 to 7 percent. And, gelling activity increases with the concentration of the coagulant and in addition, such activity also increases with the coagulant bath temperature. However, it has been found that any required bath temperature from 1° to 90° C. may be employed so long as the coating, after coagulating and just prior to casting, is in the form of a non-tacky, tough but deformable gel. And to attain such a gel condition, the time of exposure of the coating to the coagulant is preferably of the order of 0.5 to 5.0 seconds, or more, i.e., the time interval for transferring the treated coating from coagulant bath 17 to the nip 19.

The surface temperature of the casting drum 20 is preferably from 80° C. to 100° C. during the drying cycle for producing the cast-surfaced coated paper having unusually high brightness and opacity and high gloss of this invention, although temperatures ranging from 65° C. to as high as 105° C. have been used without harmful results. It has been found that temperatures approaching 90-100° C. are advantageous when the more active coagulants are employed.

Ordinarily, after the paper web 11, the coating of which has been gelled by coagulation, has been maintained in contact with the drum 20 until dry, the paper is readily stripped off the drum 20 by roll 21. As previously set forth, drum 20 preferably has a silicone resin surface but, during some operations in accordance with this invention, it was found that an ordinary metal drum such as a chromium surfaced drum could be utilized and that satisfactory release of the coating was obtained. Presumably, the coating in its gelled condition becomes so stabilized at times that it separates completely from the smoothing, clean surface drum member and is readily separated therefrom by roll 21.

As previously pointed out, a small amount of the coagulant solution may accumulate as a pool in the nip 19 between the press roll 18 and the casting surface 20. While it has been found that such a pool merely consists of clear, excess coagulant that is squeezed from the surface of the coating at the casting nip, it may, nevertheless, be desired in some operations to provide a rotating brush or a felt covered roll 27 between the nip 19 and tension roll 21 for maintaining a clean casting surface, substantially free of coagulant solution. In addition, it is preferable that the coagulant in the bath 17 be recirculated by any well known means during operations to maintain uniformity of the coagulant in the bath.

While the methods, apparatus and products herein described are for the purpose of illustration only, it is to be understood that the present invention includes all modifications and equivalents which fall within the scope of the invention which is defined by the appended claims.

What is claimed is:

1. In the coating of paper to provide a cast-surfaced mineral coated paper having unusually high brightness and opacity and high gloss with enhanced affinity for receiving printing and the like, the process which comprises the steps of applying and distributing a predetermined

and metered quantity of fluent mineral coating consisting essentially of an aqueous suspension of pigment and adhesive material to form a substantially smooth surface coating on the paper, bringing the coated surface of

5 said paper into contact with an adhesive coagulating electrolyte while said coating is still fluent on said paper to progressively convert said adhesive into a substantially tough deformable gel while maintaining a substantially uniform and smooth surfaced layer of coating, 10 bringing said coated surface of said paper into contact with a substantially smooth casting surface after said adhesive has been converted to said tough deformable gel, and drying said coating while said coating is in contact with said substantially smooth casting surface, and 15 removing said coated paper from said casting surface.

2. In the manufacture of cast-surfaced mineral coated paper having improved optical properties and enhanced affinity for printing inks, the steps comprising progressively coagulating the coating while still mobile and fluent 20 and deformable on the paper by direct contact with a coagulating electrolyte to stabilize the coating against adhesion to the surface of a casting surface, thereafter bringing said coating while so stabilized in intimate contact with said casting surface and drying said coating 25 on said casting surface, separating said coating from said casting surface.

3. The process of making cast-surfaced mineral coated paper having unusually high brightness and opacity and high gloss which comprises applying to a web of paper 30 a coating color consisting essentially of an aqueous suspension of pigment and adhesive material, said coating color having from about 45% to about 65% total solids and having said adhesive present in an amount between about 12% and about 20% of said solids, progressively coagulating said coating to form a substantially non-tacky tough deformable gel by contacting said coating color with a water solution of an adhesive coagulating electrolyte, and thereafter bringing said coating in contact with a casting surface.

4. In the coating of paper to provide a cast-surfaced mineral coated paper having unusually high brightness and opacity and high gloss with enhanced affinity for receiving printing and the like, the process which comprises the steps of applying an aqueous suspension of pigment and adhesive material of approximately 45% to 45% solids content to the paper in an initially fluent and deformable condition to form a coating thereon, stabilizing said coating against adhesion to the surface of a heated casting surface by progressively coagulating said coating with a coagulating electrolyte sufficiently to form a non-tacky tough deformable gel, thereafter bringing said coating in intimate contact with said casting surface, drying said coating against said casting surface, and withdrawing said paper from said casting surface with separation of the coating therefrom.

5. The process of producing cast-surfaced mineral coated paper of the character described comprising applying to the surface of a web of paper a coating color consisting essentially of an aqueous suspension of pigment and adhesive material, said coating color having from about 45% to about 65% total solids and having said adhesive present in an amount between about 12% and about 20% based on the weight of said total solids, said adhesive being selected from the group consisting of casein and soya protein and mixtures thereof with latex, and after application of said coating color progressively coagulating said adhesive to a tough deformable gel by contacting said coating color with a water solution of a coagulating agent selected from the group consisting of soluble calcium, zinc, barium, lead and aluminum salts of formic, acetic, citric, tartaric, lactic, hydrochloric and sulfuric acids, squeezing off the excess solution, thereafter bringing said coating in intimate contact with a heated smoothly finished casting surface, drying said coating 65 against said casting surface, and withdrawing said paper

70

from said casting surface with substantially complete separation of the coating therefrom.

6. Process as defined in claim 5, in which the coagulation agent is calcium formate.

7. Process as defined in claim 5, in which the coagulation agent is aluminum sulfate.

8. Process as defined in claim 5, in which the coagulation agent is calcium lactate.

9. Cast surfaced coated paper produced in accordance with the process of claim 5.

10. The process of producing cast-surfaced mineral coated paper of the character described comprising applying to the surface of a web of paper a coating color consisting essentially of an aqueous suspension of pigment and adhesive material, said coating color having from about 45% to about 65% total solids and having said adhesive present in an amount between about 12% and about 20% based on the weight of said total solids, and after application of said coating color progressively coagulating said adhesive to a tough deformable gel by contacting said coating color with a water solution of a coagulating agent selected from the group consisting of soluble polyvalent metal salts of formic, acetic, citric, tartaric, lactic, hydrochloric and sulfuric acids, squeezing off the excess solution, thereafter bringing said coating in intimate contact with a heated smoothly finished casting surface, drying said coating against said casting surface, and thereafter withdrawing said paper from said casting surface with substantially complete separation of the coating therefrom.

11. Process as defined in claim 10, in which the coagulation agent is cadmium sulfate.

12. Process as defined in claim 10, in which the coagulation agent is zinc acetate.

13. Process as defined in claim 10, in which the coagulating agent is a mixture of calcium formate and zinc acetate.

14. In the cast-surfaced coating of paper of the character described to produce surface characteristics adapted for receiving printing and the like, the method of forming a smooth surface on a layer of coating composition applied to paper which comprises the steps of stabilizing said coating prior to drying thereof against adhesion to the surface of a heated casting surface by progressively coagulating said coating with a coagulating electrolyte sufficiently to form a non-tacky tough deformable gel, thereafter bringing said coating in intimate contact with said casting surface, drying said coating against said casting surface, and withdrawing said paper from said casting surface with substantially complete separation of the coating therefrom.

15. The process of making cast-surfaced mineral coated paper having unusually high brightness and opacity and high gloss which comprises applying to a web of paper a fluent mineral coating color consisting essentially of an aqueous suspension of pigment and adhesive material, said coating color having from about 45% to about 65% total solids and having said adhesive present in an amount between about 12% and about 20% of said solids, said adhesive selected from the group consisting of casein and soya protein and mixtures thereof with latex, progressively coagulating said coating to form a substantially non-tacky tough deformable gel by contacting said coating color with a water solution of an adhesive coagulating electrolyte, and thereafter bringing and drying said coating in intimate contact with a casting surface.

References Cited in the file of this patent

UNITED STATES PATENTS

|           |              |               |
|-----------|--------------|---------------|
| 2,304,818 | Grupe        | Dec. 15, 1942 |
| 2,678,890 | Leighton     | May 18, 1954  |
| 2,772,184 | Wolfe        | Nov. 27, 1956 |
| 2,780,563 | Frost et al. | Feb. 5, 1957  |
| 2,790,736 | McLaughlin   | Apr. 30, 1957 |